

[54] **DEHYDRATION PROCESS TO IMPART WRINKLE RESISTANCE TO CELLULOSE-CONTAINING FIBROUS MATERIALS**[75] Inventors: **Russel M. Kullman**, Metairie; **Robert M. Reinhardt**, New Orleans, both of La.[73] Assignee: **The United States of America as represented by the Secretary of Agriculture**, Washington, D.C.

[22] Filed: July 25, 1972

[21] Appl. No.: 274,949

[52] U.S. Cl. .... 8/186; 8/187; 8/116.4

[51] Int. Cl.<sup>2</sup> .... D06M 13/34

[58] Field of Search .... 8/116.4, 189, 181-187, 8/149.2

[56] **References Cited**

## UNITED STATES PATENTS

3,224,926 12/1965 Bernardin .... 8/116.4 X

|           |         |                                 |
|-----------|---------|---------------------------------|
| 3,264,054 | 8/1966  | Reinhardt et al. .... 8/116.4 X |
| 3,278,470 | 10/1966 | Henshall et al. .... 8/116.4 X  |
| 3,285,690 | 11/1966 | Cooper et al. .... 8/187 x      |
| 3,312,521 | 4/1967  | Stenner .... 8/116.4            |
| 3,350,162 | 10/1967 | Beck .... 8/116.4 X             |
| 3,371,983 | 3/1968  | Barber et al. .... 8/116.4      |
| 3,527,558 | 9/1970  | Tomasino et al. .... 8/189      |
| 3,533,728 | 10/1970 | Shippee et al. .... 8/189       |
| 3,653,805 | 4/1972  | Gamarra et al. .... 8/149.2 X   |
| 3,660,013 | 5/1972  | Payet et al. .... 8/149.2 X     |
| 3,706,526 | 12/1972 | Swidler et al. .... 8/149.2 X   |

Primary Examiner—Stephen J. Lechert, Jr.  
 Attorney, Agent, or Firm—M. Howard Silverstein; Max D. Hensely

[57] **ABSTRACT**

Crosslinking formulations are applied to cotton and other cellulose-containing textiles and made to react by dehydrating the impregnated textile at ambient temperatures and pressures.

**30 Claims, No Drawings**

**DEHYDRATION PROCESS TO IMPART WRINKLE  
RESISTANCE TO CELLULOSE-CONTAINING  
FIBROUS MATERIALS**

A non-exclusive, irrevocable, royalty-free license in the invention herein described throughout the world for all purposes of the United States Government, with the power to grant sublicenses for such purposes, is hereby granted to the Government of the United States of America.

This invention relates to the chemical finishing of textiles. More particularly, this invention relates to a process for chemical finishing of cellulose-containing fibrous materials to effect crosslinking and improvement in wrinkle resistance. Specifically, this invention relates to a new method of curing a cellulose-containing textile material which has been impregnated with certain crosslinking formulations, the novelty comprising removing moisture upon exposure of the impregnated material to an unheated, dehydrating atmosphere at ambient temperatures and pressures thereby generating the conditions necessary for reaction of a crosslinking reagent with the cellulose and enhancing wrinkle resistance. Hereinafter this novel method of textile processing is referred to as dehydration curing.

**THE PRIOR ART**

There are several processes for producing improved wrinkle resistance in cellulosic materials. That most commonly employed is the pad-dry-cure process. Curing is accomplished in this type of process by subjecting the impregnated material to a strongly heated atmosphere (usually 140° to 180°C). Another method of treatment employed is the mild cure finishing process wherein the curing is accomplished with heating at mild temperatures of 60° to 100°C, so that moisture content within the fiber is critically controlled. This method requires precise adjustment of the moisture content in the material being treated.

In another process of the prior art for improved wrinkle resistance, the fibrous material is cured by maintaining a moist condition at about 25°C for from 4 to 30 hours, then neutralizing, washing, and drying. Wet finishing treatments also are known wherein the reaction of the cellulosic fiber proceeds while the fiber is maintained at a level of swelling which is controlled by composition of the treatment bath.

Various modifications have been reported in the literature to achieve improved wet wrinkle resistance or improved wet and dry wrinkle resistance wherein the fibrous material must be (1) exposed to elevated temperatures during curing (considerably higher than ambient room temperatures), as in the pad-dry-cure and mild cure processes; or (2) maintained at a predetermined moisture level during curing, as in moist or wet processes.

Among the advantages of the present invention over the prior art are the savings of heat energy afforded, the greater comfort of workers by the absence of elevated temperatures usually encountered in finishing plants, and particularly the superior levels of wrinkle resistance and chlorine resistance of fabrics treated by the process. The value of wrinkle resistance in textile materials is widely recognized by those skilled in the art. It has been estimated that current annual production in the United States alone of fabric for use in durable press and wrinkle resistant products is about three billion yards.

The main object of the present invention is to provide a process for imparting improved wrinkle resistance by the chemical finishing of cellulose-containing textiles without subjecting the textile to elevated temperatures, without the need of maintaining moisture content in the fibers at critical levels, and without the need for controlling swelling of the fibers through adjustment of the composition of the treatment bath.

We have unexpectedly discovered that reaction between certain crosslinking formulations and cellulose-containing textiles can be effected readily by the process of our invention. Said process requires no heating during curing and no controlled levels of moisture nor swelling of the fiber. By the process of this invention the fibrous material can be dried and cured by treatment with unheated dehydrating air at ambient temperatures and pressures after impregnating the cellulose-containing textile with the crosslinking formulation and removing the excess by conventional squeeze-roll techniques.

The instant invention can best be described as a process for imparting wrinkle resistance to cellulose-containing fibrous material, the process comprising:

- a. impregnating the cellulose-containing fibrous material with a formulation containing about from 5 to 25 weight percent of a crosslinking agent selected from the group consisting of glyoxal, formaldehyde, dimethylol dihydroxyethyleneurea, and dimethylol methyl carbamate and about from 0.1 to 1.2 weight percent of an inorganic acid catalyst selected from the group consisting of hydrochloric acid, hydrobromic acid, sulfuric acid, sulfurous acid, phosphoric acid, phosphorous acid, nitric acid, and nitrous acid,
- b. removing the excess quantity of formulation to obtain a wet pickup of about 60 to 100 percent, and
- c. exposing the fibrous material of step (b) to a dehydrating atmosphere at ambient temperatures and pressures, for periods of time about from 30 minutes to 24 hours, the longer periods of time being employed with a static dehydrating atmosphere and the shorter periods of time being employed with a dynamic dehydrating atmosphere.

An optional step can be inserted between above steps (b) and (c) wherein the wet fibrous material of step (b) is dried to a moisture content intermediate between that of the wet fabric and complete dryness by passing the impregnated material through a conventional drying oven. The time of dehydration treatment necessary to produce a given level of wrinkle resistance in fabric can be markedly decreased by such a partial drying step.

The products produced by the process are part of this invention. These have outstanding qualities both high dry and wet wrinkle resistance and high levels of resistance to damage due to retained chlorine.

By the process of the present invention fibrous material to be employed therein may be in the form of fibers, yarns, and fabrics; either woven or knitted. The material may be composed entirely of cellulosic fibers, either natural or regenerated, or may be composed of said cellulosics as components with other non-cellulosic natural and synthetic components.

**PREFERRED REAGENTS**

Preferred reagents for use in the process of this invention are difunctional and polyfunctional chemical agents that react with the hydroxyl groups of cellulose

under acidic conditions. These agents include formaldehyde adducts (methylol derivatives) of nitrogenous compounds, such as dimethylol alkyl carbamates, dimethylol dihydroxyethyleneurea, dimethylol propyleneureas, and the like; modified methylol agents, such as N-methoxymethyl, N-isopropoxymethyl, and N-acetoxymethyl derivatives, and the like; monoaldehydes, such as formaldehyde; and dialdehydes, such as glyoxal. The concentration of the crosslinking chemical agent employed in the process may be varied in the range of from about 2.5 percent to 35 percent by weight, based on the total weight of the finishing solution. The preferred range is from about 10 to about 20 percent.

The catalyst employed in the formulation may be an organic acid, a strong Lewis acid, or a mineral acid. The preferred catalyst is an inorganic acid such as hydrochloric, sulfuric, nitric acid and the like. Concentration of the catalyst in the treating solution may be varied from about 0.025 to about 2.5 weight percent but we have found that the range of 0.1 to 1.2 weight percent to be preferred in this invention.

Additives known to those skilled in the art may be used in the treating solution for supplementary effects such as softness of hand and the like.

#### THE DEHYDRATION STEP

Dehydration curing by the process of this invention is carried out after impregnation of the fibrous material with a solution containing the chemical crosslinking agent and catalyst, or alternately, after partially drying the impregnated material. Impregnation may be accomplished by any suitable means. For fabric treatments, impregnation is most commonly accomplished by immersing the fabric in the treatment solution, then squeezing out excess solution by passing through pad rolls which also facilitates uniform penetration and distribution of the treatment solution within the fibrous material. Based upon the dry weight of the material, a wet pickup of about 60 to 100 percent is preferred.

The fibrous material may then, as shown in the following Examples, be partially dried before curing under ambient pressures and temperatures. The material is heated for about from 1.5 to 7 minutes at a temperature sufficient to partial dry the material, e.g., about 60°C.

Curing conditions which may be employed in the process of this invention include exposure of the suitably impregnated fibrous material to a static or a dynamic (moving) dehydrating atmosphere under ambient pressures and temperatures of about from 20° to 30°C, for periods of about from 30 minutes to 24 hours. Time required can vary depending upon selection of a static or dynamic dehydrating atmosphere. An after-wash of the treated fabric by any conventional washing procedure is done after curing to remove residual catalyst, unused reactant, and byproducts. After-washing

may be omitted with some catalysts as the cured material regains moisture on removal from the dehydrating atmosphere, said moisture may be sufficient to dilute and render any remaining catalyst or acidic material innocuous.

In summary, this invention provides a process (and products by said process) for finishing fibrous materials containing a cellulosic component to produce a product with improved wrinkle resistance. Wrinkle resistance as a useful fabric property is well known and is a necessity for durable press garments that are in such demand by American and other consumers. The curing treatment of the process is carried out in the presence of an unheated, dehydrating atmosphere. The process may be summarized as:

- a. impregnating the fibrous material containing a cellulosic component to about 60-100 percent wet pickup of a solution containing 5-25 percent of a chemical agent capable of crosslinking the cellulosic component, and an inorganic acid catalyst; and
- b. exposing the impregnated material to a static or a dynamic unheated dehydrating atmosphere at ambient temperatures and pressures, for periods of time sufficient to effect the crosslinking reaction to produce a fibrous material having improved wrinkle resistance.

The following examples are set forth to illustrate certain significant aspects of the invention, and should not be construed as limiting the invention in any manner whatever.

#### EXAMPLE 1

35 Swatches of cotton printcloth were padded to about 90 percent wet pickup with an aqueous solution containing 15 percent (wt./wt.) of dimethylol methyl carbamate and 0.4 percent (wt./wt.) of hydrogen chloride (from hydrochloric acid). These swatches were divided into Groups A, B, and C. Samples from each group 40 were partially dried in a 60°C atmosphere for 1.5, 3, 5, and 7 minutes which reduced the moisture contents to about 40, 18, 4, and 3 percent, respectively. Group A samples, A-1.5, A-3, A-5, and A-7, immediately after partial drying were neutralized in a dilute solution (approximately 1 percent, wt/wt) of sodium carbonate, then washed and dried. Group B samples, B-1.5, B-3, B-5, and B-7, after partial drying were placed in a reaction chamber in contact with a dehydrating atmosphere (static conditions, normal pressures) over P<sub>2</sub>O<sub>5</sub> desiccant at 25°C for 22 hours, removed, neutralized in the sodium carbonate solution, then washed and dried. Group C samples, C-1.5, C-3, C-5, and C-7, after partial drying were immediately sealed in plastic bags and maintained at constant moisture levels for 22 hours at 50 25°C, removed, neutralized in the sodium carbonate solution, then washed and dried. Results are shown in Table 1.

TABLE 1

| Sample | Partial drying (min. at 60°C) | % Moisture content after partial drying | % HCHO | % N  | WRA, W+F deg | % Strength retention in Cl-scorch test |
|--------|-------------------------------|-----------------------------------------|--------|------|--------------|----------------------------------------|
|        |                               |                                         |        |      | Dry      Wet |                                        |
| A-1.5  | 1.5                           | 40                                      | 0.21   | 0.13 | 183      175 | 3                                      |
| A-3    | 3                             | 18                                      | 0.50   | 0.12 | 197      170 | 3                                      |
| A-5    | 5                             | 4                                       | 3.46   | 0.98 | 248      259 | 23                                     |
| A-7    | 7                             | 3                                       | 3.59   | 1.16 | 261      275 | 81                                     |
| B-1.5  | 1.5                           | 40                                      | 5.30   | 1.31 | 285      308 | 99                                     |
| B-3    | 3                             | 18                                      | 4.92   | 1.38 | 282      308 | 100                                    |

TABLE I-continued

| Sample | Partial drying (min. at 60°C) | % Moisture content after partial drying | % HCHO | % N  | WRA, W+F deg<br>Dry | WRA, W+F deg<br>Wet | % Strength retention in Cl-scorch test |
|--------|-------------------------------|-----------------------------------------|--------|------|---------------------|---------------------|----------------------------------------|
| B-5    | 5                             | 4                                       | 4.42   | 1.27 | 272                 | 290                 | 95                                     |
| B-7    | 7                             | 3                                       | 4.32   | 1.40 | 261                 | 288                 | 96                                     |
| C-1.5  | 1.5                           | 40                                      | 0.73   | 0.31 | 189                 | 180                 | 2                                      |
| C-3    | 3                             | 18                                      | 1.56   | 0.44 | 192                 | 254                 | 7                                      |
| C-5    | 5                             | 4                                       | 3.30   | 1.03 | 269                 | 282                 | 36                                     |
| C-7    | 7                             | 3                                       | 3.87   | 1.10 | 270                 | 278                 | 65                                     |

These data show that samples of Group B, the process of the present invention, are superior in reaction efficiency as seen by high nitrogen and formaldehyde contents, high wet and dry wrinkle recovery angles, and high levels of strength retention in the chlorination-scorch test (AATCC Test Method 92-1967, American Association of Textile Chemists and Colorists). The data also reveal that partial drying to too low a level of moisture content prior to exposure to an unheated dehydrating atmosphere gives a lower wrinkle recovery than do treatments in which samples with higher moisture levels are exposed to the unheated dehydrating atmosphere. Furthermore, prevention of moisture loss during the curing reaction as in the treatments of Group C does not produce comparably high levels of wet wrinkle recovery nor of strength retention in the chlorination-scorch test.

## EXAMPLE 2

Swatches of cotton printcloth were padded to about 90 percent wet pickup with a solution containing 10 percent (wt./wt.) of formaldehyde and 0.4 percent (wt./wt.) of hydrogen chloride. Four samples were partially dried as in Example 1 for 1.5, 3, 5, and 7 minutes, respectively. These samples were coded D-1.5, D-3, D-5, and D-7. In addition, one sample coded D-0, was not partially dried. The samples were treated in a dehydration chamber over  $P_2O_5$  desiccant at 25°C for 20 hours, removed, washed, and dried. Results are shown in Table II.

TABLE II

| Sample | % HCHO | WRA, W+F, deg. |     |
|--------|--------|----------------|-----|
|        |        | Dry            | Wet |
| D-0    | 0.82   | 247            | 276 |
| D-1.5  | 1.18   | 287            | 286 |
| D-3    | 1.21   | 284            | 289 |
| D-5    | 1.17   | 283            | 279 |
| D-7    | 1.39   | 288            | 281 |

From these data it is shown that the new process for producing improved wrinkle resistance is effective with monoaldehyde crosslinking agents.

## EXAMPLE 3

A swatch of cotton printcloth was padded to about 100% wet pickup with a solution containing 11.7 percent (wt./wt.) of glyoxal and 0.4 percent (wt./wt.) of hydrogen chloride. The swatch was partially dried for 3 minutes in a 60°C atmosphere, placed in the dehydration chamber over  $P_2O_5$  desiccant at 25°C for 20 hours, removed, washed, and dried. Dry wrinkle resistance was 234°.

This shows that the new process for producing improved wrinkle resistance is effective with dialdehyde crosslinking agents.

## EXAMPLE 4

15 Swatches of cotton printcloth were padded to about 90 percent wet pickup with a solution containing 15 percent (wt./wt.) of dimethylol methyl carbamate and 0.4 percent (wt./wt.) of hydrogen chloride. These swatches were divided into Groups E and F and partially dried in a 60°C atmosphere for 3 minutes (about 20 18 percent moisture content). Group E swatches, E-½, E-¼, E-1, E-2, and E-3, after partial drying were placed in a dehydration chamber over  $P_2O_5$  desiccant. An inlet and outlet connection on the chamber allowed unheated, anhydrous air to be passed into, through, and out of the chamber during dehydration of the E samples. Ambient air at 25°C was made anhydrous by bubbling through concentrated sulfuric acid and used for the treatment. E samples were treated by this procedure for ½, ¼, 1, 2, and 3 hours at 25°C. They were coded E-½, E-¼, E-1, E-2, and E-3, respectively. After the treatment, they were removed, neutralized in sodium carbonate solution as in Example 1, then washed and dried. Samples F-1, F-2, and F-3 were placed in the 35 dehydration chamber over  $P_2O_5$  desiccant at 25°C for 1, 2, and 3 hours, respectively as done for B samples in Example 1. They were then removed, neutralized in the sodium carbonate solution as in Example 1, washed and dried. Results are shown in Table III.

TABLE III

| Sample    | WRA, W+F, deg.<br>Dry | Sample    | WRA, W+F, deg.<br>Dry |
|-----------|-----------------------|-----------|-----------------------|
| Untreated | 187                   | Untreated | 187                   |
| E-½       | 211                   | —         | —                     |
| E-¼       | 253                   | —         | —                     |
| E-1       | 270                   | F-1       | 204                   |
| E-2       | 286                   | F-2       | 222                   |
| E-3       | 281                   | F-3       | 233                   |

40 From data in this table, it is seen that development of dry wrinkle recovery by the new process may be accelerated greatly by dynamic conditions in which anhydrous air at 25°C is passed through the reaction chamber during the dehydration curing treatment.

## EXAMPLE 5

45 A swatch of cotton printcloth was padded to about 100 percent wet pickup with a solution containing 15 percent (wt./wt.) of dimethylol methyl carbamate and 0.4 percent (wt./wt.) of hydrogen chloride. The wet-impregnated fabric was placed in a dehydration chamber as in Example 4 but in the absence of  $P_2O_5$ . Ambient air at 28°C was made anhydrous by passing through 50 a heat exchange coil immersed in a dry ice (solid  $CO_2$ )-acetone bath at -67°C such that moisture in the air was condensed, frozen, and thus removed. The anhydrous air was then passed through glass coils to achieve a

temperature of 28°C and thence into, through, and out of the dehydration chamber during dehydration of the sample. The sample was removed after 3 hours then washed and dried. The relative humidity in the dehydration chamber prior to placing of the wet-impregnated sample and prior to passing through anhydrous air was 65 percent and the temperature was 28°C. In the following table are listed relative humidities before and during the dehydration process.

TABLE IV

| Time after sample insertion in chamber | Chamber relative humidity % | Chamber temperature, °C |
|----------------------------------------|-----------------------------|-------------------------|
| 0                                      | 65                          | 28                      |
| 15 minutes                             | 78.5                        | 28                      |
| 45 minutes                             | 80.5                        | 28                      |
| 3 hours                                | 52                          | 28                      |

The dry wrinkle resistance of the finished fabric was 262° and the wet wrinkle resistance was 264°.

The initial increase in relative humidity is due to the moisture introduced by the wet-impregnated fabric. During the course of reaction between the finished agent and cellulose more water is produced which also contributes to increased humidity. This is seen in the following equation which represent the crosslinking reaction that produces wrinkle resistance.



Dehydration of the fabric and the reaction has occurred to a sufficient extent after three hours at a constant temperature to produce a wrinkle resistant fabric. The relative humidity after three hours reflects that the dehydration of the fabric and the reaction have approached completion.

## EXAMPLE 6

A swatch of a fabric comprised of an equiweight mixture of polyester and cotton was padded to about 80 percent wet pickup with a solution containing 25 percent (wt/wt) of dimethylol methyl carbamate and 0.6 percent (wt/wt) of hydrogen chloride. The swatch labelled G, was partially dried for 3 minutes in a 60°C atmosphere, placed in the dehydration chamber over  $\text{P}_2\text{O}_5$  desiccant at 25°C for 1½ hours as Sample E in Example 4 with anhydrous air flowing into, through, and out of the chamber. After removal and washing the sample was tumble dried in an automatic home dryer, then evaluated for durable press appearance using the AATCC 3-dimensional standards.

An untreated swatch, labelled H, of the same fabric containing equiweight mixtures of polyester and cotton after being washed and tumble dried in the same manner as Sample G was also evaluated with the AATCC 3-dimensional standards.

Sample G and H were also tested for wrinkle recovery and results are shown in Table V.

TABLE V

| Sample | WRA, W+F, deg.<br>Dry | WRA, W+F, deg.<br>Wet | Durable Press Rating<br>after tumble drying |
|--------|-----------------------|-----------------------|---------------------------------------------|
| G      | 259                   | 290                   | 3.6                                         |
| H      | 235                   | 264                   | 2.0                                         |

This shows that the new process is effective in improving durable press performance, as measured by improvement in dry and wet wrinkle recovery and smoothness appearance as measured by the durable press rating of fabrics containing up to 50 percent by weight of a cellulosic component.

## EXAMPLE 7

Four swatches of cotton printcloth were labelled I, J, K, and L respectively. Swatches were padded to about 90 percent wet pickup with solutions as identified in the following data:

| Swatch | % HCl in treatment solution | % Dimethylol methyl carbamate in treatment solution |
|--------|-----------------------------|-----------------------------------------------------|
| I      | 0.14                        | 5                                                   |
| J      | 0.28                        | 10                                                  |
| K      | 0.59                        | 25                                                  |

Swatch L was not treated. Swatches I, J, and K were partially dried for 3 minutes in a 60°C atmosphere, placed in the dehydration chamber over  $\text{P}_2\text{O}_5$  desiccant at 25°C for 1½ hours as Sample E in Example 4 with anhydrous air flowing into, through, and out of the chamber. After removal, samples I, J, K, and L were washed, tumble dried and evaluated for wrinkle recovery. Results are shown in Table VI.

TABLE VI

| Sample | WRA, dry | Durable Press Rating after Tumble Drying |
|--------|----------|------------------------------------------|
| I      | 225      | 2.7                                      |
| J      | 259      | 3.7                                      |
| K      | 270      | 4.5                                      |
| L      | 206      | 1.0                                      |

Improvement in wrinkle recovery and smoothness appearance was achieved in each instance over a wide range of concentration of catalyst and crosslinking agent by use of this new process over the untreated sample (Sample L).

## EXAMPLE 8

Swatches of cotton printcloth, labelled M and N were padded to about 90 percent wet pickup and aqueous solutions identified below:

| Swatch | % $\text{H}_2\text{SO}_4$ | % DMDHEU <sup>11</sup> |
|--------|---------------------------|------------------------|
| M      | 0.6                       | 15                     |
| N      | 1.2                       | 15                     |

<sup>11</sup>DMDHEU is dimethylol dihydroxyethyleneurea, a tetrafunctional crosslinking agent.

The swatches were partially dried for 3 minutes in a 60°C atmosphere, placed in the dehydration chamber over  $\text{P}_2\text{O}_5$  desiccant at 25°C for 1½ hours as Sample E in Example 4 with anhydrous air flowing into, through

and out of the chamber. After removal, the samples were washed, dried, and evaluated. Results are listed in Table VII.

TABLE VII

| Sample        | WRA, dry | Durable Press Rating<br>after Tumble drying |
|---------------|----------|---------------------------------------------|
| M             | 266      | 3.7                                         |
| N             | 291      | 4.6                                         |
| L (untreated) | 206      | 1.0                                         |

This demonstrates that the process is useful with other mineral catalysts and tetrafunctional crosslinking agents.

We claim:

1. A process for imparting wrinkle resistance to cellulose-containing fibrous material comprising:
  - a. impregnating the cellulose-containing fibrous material with a formulation containing about from 2.5 to 35 weight percent of a crosslinking agent and about from 0.025 to 25 weight percent of an inorganic acid catalyst,
  - b. removing the excess quantity of formulation to obtain a wet pickup of about 60 to 100 weight percent, and
  - c. exposing the fibrous material of step (b) to a dehydrating atmosphere at ambient temperatures and pressures, for periods of time about from 30 minutes to 24 hours.
2. A process for imparting wrinkle resistance to cellulose-containing fibrous material comprising:
  - a. impregnating the cellulose-containing fibrous material with a formulation containing about from 2.5 to 35 weight percent of a crosslinking agent selected from the group consisting of:
    - glyoxal
    - formaldehyde
    - dimethylol dihydroxyethyleneurea, and
    - dimethylol methyl carbamate
 and about from 0.025 to 2.5 weight percent of an inorganic acid catalyst selected from the group consisting of:
    - hydrochloric acid
    - hydrobromic acid
    - sulfuric acid
    - sulfurous acid
    - phosphoric acid
    - phosphorous acid
    - nitric acid, and
    - nitrous acid,
  - b. removing the excess quantity of formulation to obtain a wet pickup of about 60 to 100 weight percent, and
  - c. exposing the fibrous material of step (b) to a dehydrating atmosphere at ambient temperatures and pressures, for periods of time about from 30 minutes to 24 hours, the longer periods of time being employed with a static dehydrating atmosphere and the shorter periods of time being employed with a dynamic dehydrating atmosphere.
3. The process of claim 2 wherein the crosslinking agent is glyoxal.
4. The process of claim 2 wherein the crosslinking agent is formaldehyde.
5. The process of claim 2 wherein the crosslinking agent is dimethylol dihydroxyethyleneurea.

6. The process of claim 2 wherein the crosslinking agent is dimethylol methyl carbamate.
7. The process of claim 2 wherein the inorganic acid catalyst is hydrochloric acid.
8. The process of claim 2 wherein the inorganic acid catalyst is hydrobromic acid.
9. The process of claim 2 wherein the inorganic acid catalyst is sulfuric acid.
10. The process of claim 2 wherein the inorganic acid catalyst is sulfurous acid.
11. The process of claim 2 wherein the inorganic acid catalyst is phosphoric acid.
12. The process of claim 2 wherein the inorganic acid catalyst is phosphorous acid.
13. The process of claim 2 wherein the inorganic acid catalyst is nitric acid.
14. The process of claim 2 wherein the inorganic acid catalyst is nitrous acid.
15. A process for imparting wrinkle resistance to cellulose-containing fibrous material comprising:
  - a. impregnating the cellulose-containing fibrous material with a formulation containing about from 2.5 to 35 weight percent of a crosslinking agent and about from 0.025 to 2.5 weight percent of an inorganic acid catalyst,
  - b. removing the excess quantity of formulation to obtain a wet pickup of about 60 to 100 weight percent,
  - c. heating the fibrous material for about from 1.5 to 7 minutes at a temperature sufficient to partially dry said material, and
  - d. exposing the fibrous material of step (c) to a dehydrating atmosphere at ambient temperatures and pressures.
16. A process for imparting wrinkle resistance to cellulose-containing fibrous material, comprising:
  - a. impregnating the cellulose-containing fibrous material with a formulation containing about from 2.5 to 35 weight percent of a crosslinking agent selected from the group consisting of:
    - glyoxal
    - formaldehyde
    - dimethylol dihydroxyethyleneurea, and
    - dimethylol methyl carbamate
 and about from 0.025 to 2.5 weight percent of an inorganic acid catalyst selected from the group consisting of:
    - hydrochloric acid
    - hydrobromic acid
    - sulfuric acid
    - sulfurous acid
    - phosphoric acid
    - phosphorous acid
    - nitric acid, and
    - nitrous acid
  - b. removing the excess quantity of formulation to obtain a wet pickup of about 60 to 100 weight percent, and
  - c. heating the fibrous material for about from 1.5 to 7 minutes at a temperature of about 60° C.
  - d. exposing the fibrous material of step (c) to a dehydrating atmosphere at ambient temperatures and pressures for periods of time about from 30 minutes to 24 hours.
17. The process of claim 16 wherein the crosslinking agent is glyoxal.
18. The process of claim 16 wherein the crosslinking agent is formaldehyde.

11

19. The process of claim 16 wherein the crosslinking agent is dimethylol dihydroxyethyleneurea.

20. The process of claim 16 wherein the crosslinking agent is dimethylol methyl carbamate.

21. The process of claim 16 wherein the inorganic acid catalyst is hydrochloric acid.

22. The process of claim 16 wherein the inorganic acid catalyst is hydrobromic acid.

23. The process of claim 16 wherein the inorganic acid catalyst is sulfuric acid.

24. The process of claim 16 wherein the inorganic acid catalyst is sulfurous acid.

12

25. The process of claim 16 wherein the inorganic acid catalyst is phosphoric acid.

26. The process of claim 16 wherein the inorganic acid catalyst is phosphorous acid.

27. The process of claim 16 wherein the inorganic acid catalyst is nitric acid.

28. The process of claim 16 wherein the inorganic acid catalyst is nitrous acid.

10 29. The product produced by the process of claim 2.

30. The product produced by the process of claim 16.

\* \* \* \* \*

15

20

25

30

35

40

45

50

55

60

65